

May 4, 1971

J. A. ZIC ET AL

3,577,283

METHOD OF CASEHARDENING VANADIUM AND VANADIUM ALLOYS

Filed March 7, 1969



DPH No. (10 kg Load)

Inventors

Ross M. Mayfield  
John A. Zic  
George F. Hill

Ronald G. Goodman  
Attorney

## 1

3,577,283

### METHOD OF CASEHARDENING VANADIUM AND VANADIUM ALLOYS

John A. Zic, Oak Lawn, and George F. Hill, Chicago, Ill., and Ross M. Mayfield, deceased, late of Glen Ellyn, Ill., by Georgia P. Mayfield, sole heir, Glen Ellyn, Ill., assignors to the United States of America as represented by the United States Atomic Energy Commission

Filed Mar. 7, 1969, Ser. No. 805,384

Int. Cl. C21d 1/74

U.S. CL. 148—20.3

1 Claim 10

#### ABSTRACT OF THE DISCLOSURE

A method of casehardening vanadium and vanadium alloys consisting predominantly of vanadium by heating the material briefly at 1100 to 1300° C. in an atmosphere of argon saturated with water vapor.

#### CONTRACTUAL ORIGIN OF THE INVENTION

The invention described herein was made in the course of, or under, a contract with the United States Atomic Energy Commission.

#### BACKGROUND OF THE INVENTION

Metals such as titanium, zirconium, vanadium and tantalum are very resistant to attack by certain chemical agents while having relatively high melting points. These metals, and alloys thereof, are, therefore, suitable for use as materials of construction in the chemical industry. Unfortunately, these same materials are not hard enough without treatment for use where wear is a factor, such as in valves, nozzles, orifice plates and the like.

Various procedures are known for casehardening these materials, all of which involve controllably diffusing oxygen, carbon and/or nitrogen into the metal lattice. Vanadium and alloys consisting predominantly of vanadium are difficult to caseharden, because vanadium reacts quite readily with oxygen; thus attempts to caseharden vanadium usually result in oxidation of the metal rather than controlled diffusion of oxygen into the metal.

#### SUMMARY OF THE INVENTION

According to the present invention, controlled diffusion of oxygen into vanadium and vanadium alloys to obtain a hardened case is accomplished by heating the material briefly in an atmosphere of argon saturated with water vapor at 1100 to 1300° C. This procedure ensures that the material will be contacted by a limited, controllable amount of oxygen for diffusion into the case.

#### BRIEF DESCRIPTION OF THE DRAWING

The single figure of the drawing is a graph in which hardness is plotted as a function of position in test specimens which have been subjected to differing heat treatments.

#### DESCRIPTION OF THE PREFERRED EMBODIMENT

All of the test specimens employed in the tests described hereinafter were vanadium-20% titanium rods. The rods used in Examples 1-6 were 0.223" in diameter and 3 1/4" in length, while the rods used in Examples 7 and 8 were 0.218" in diameter and 2 1/2" in length. The first-mentioned rods had been rolled to a diameter of 0.260", swaged to a diameter of 0.242", annealed at 900° C. for one hour, and then centerless ground to a diameter of 0.323". A similar procedure was used to prepare the rods used in Examples 7 and 8. The original hardness of all rods was about DPH 260. In all tests, the equipment was purged with argon for five minutes

## 2

and the hardness measured on opposite sides of the rod at 1/16" intervals along the rod using a 10-kilogram weight in an Avery hardness tester.

#### Example 1

Heated at 1525° C. for one minute—total heat cycle, five minutes—cooled ten minutes in argon.

| Distance from end of rod | Diamond pyramid hardness |                      |         |
|--------------------------|--------------------------|----------------------|---------|
|                          | One side of rod          | Opposite side of rod | Average |
| 3 1/16"                  | 270                      | 309                  | 290     |
| 3 1/8"                   | 276                      | 317                  | 295     |
| 3 1/4"                   | 276                      | 294                  | 285     |
| 3 5/8"                   | 268                      | 253                  | 260     |
| 3 1/2"                   | 274                      | 240                  | 258     |
| 3 7/8"                   | 272                      | 243                  | 258     |
| 4 1/4"                   | 264                      | 245                  | 255     |
| 4 1/8"                   | 249                      | 245                  | 247     |
| 4 1/2"                   | 249                      | 245                  | 247     |
| 4 1/4"                   | 249                      | 245                  | 247     |
| 4 1/2"                   | 247                      | 245                  | 246     |
| 4 3/4"                   | 245                      | 245                  | 245     |
| 5"                       | 242                      | 245                  | 243     |

#### Example 2

Heated at 1475-1500° C. for one minute in a container having a pool of water in the bottom—total heat cycle, six minutes—quenched in the water at the bottom of the container.

| Distance from end of rod | Diamond pyramid hardness |                      |         |
|--------------------------|--------------------------|----------------------|---------|
|                          | One side of rod          | Opposite side of rod | Average |
| 3 1/16"                  | 772                      | 882                  | 822     |
| 3 1/8"                   | 946                      | 882                  | 915     |
| 3 1/4"                   | 882                      | 882                  | 882     |
| 3 5/8"                   | 920                      | 838                  | 890     |
| 3 1/2"                   | 946                      | 858                  | 903     |
| 3 7/8"                   | 858                      | 858                  | 858     |
| 4 1/4"                   | 946                      | 858                  | 903     |
| 4 1/2"                   | 882                      | 858                  | 870     |
| 4 3/8"                   | 882                      | 858                  | 870     |
| 4 1/4"                   | 858                      | 824                  | 840     |
| 4 1/2"                   | 698                      | 681                  | 690     |
| 4 3/8"                   | 698                      | 707                  | 702     |
| 4 1/2"                   | 698                      | 707                  | 702     |
| 4 1/4"                   | 542                      | 657                  | 597     |
| 4 1/2"                   | 442                      | 383                  | 410     |
| 4 3/8"                   | 351                      | 339                  | 345     |
| 4 1/2"                   | 274                      | 274                  | 274     |

#### Example 3

Heated at 1500-1520° C. for one minute—total heat cycle, four minutes—end quenched for five minutes with 745 cc./min. of water through 1/16" outlet disposed 1/8" below test specimen—shield located 1" from the water orifice to prevent splashing of water on the sides of the rod.

| Distance from end of rod | Diamond pyramid hardness |                      |         |
|--------------------------|--------------------------|----------------------|---------|
|                          | One side of rod          | Opposite side of rod | Average |
| 3 1/16"                  | 488                      | 442                  | 465     |
| 3 1/8"                   | 429                      | 450                  | 440     |
| 3 1/4"                   | 429                      | 425                  | 427     |
| 3 5/8"                   | 429                      | 397                  | 413     |
| 3 1/2"                   | 429                      | 360                  | 395     |
| 3 7/8"                   | 421                      | 366                  | 395     |
| 4 1/4"                   | 357                      | 348                  | 353     |
| 4 1/2"                   | 383                      | 348                  | 365     |
| 4 3/8"                   | 357                      | 348                  | 353     |
| 4 1/4"                   | 319                      | 348                  | 335     |
| 4 1/2"                   | 319                      | 317                  | 318     |
| 4 3/8"                   | 319                      | 274                  | 296     |
| 4 1/2"                   | 297                      | 274                  | 285     |

#### Example 4

Heated at 1400-1425° C. for one minute—total heat cycle, four minutes—end quenched for five minutes with

700 cc./min. of water through  $\frac{1}{16}$ " outlet disposed  $\frac{1}{8}$ " below test specimen. A shield was used.

| Distance from end of rod | Diamond pyramid hardness |                      |         |
|--------------------------|--------------------------|----------------------|---------|
|                          | One side of rod          | Opposite side of rod | Average |
| $\frac{1}{16}$ "         | 464                      | 464                  | 464     |
| $\frac{3}{16}$ "         | 401                      | 401                  | 401     |
| $\frac{1}{4}$ "          | 366                      | 401                  | 384     |
| $\frac{3}{8}$ "          | 366                      | 394                  | 380     |
| $\frac{1}{2}$ "          | 351                      | 380                  | 366     |
| $\frac{5}{16}$ "         | 351                      | 357                  | 354     |
| $\frac{7}{16}$ "         | 322                      | 357                  | 340     |
| $\frac{9}{16}$ "         | 317                      | 339                  | 328     |
| 1"                       | 317                      | 339                  | 328     |
| $1\frac{1}{16}$ "        | 281                      | 330                  | 305     |
| $1\frac{3}{16}$ "        | 281                      | 314                  | 298     |
| $1\frac{7}{16}$ "        | 281                      | 306                  | 294     |
| 2"                       | 274                      | 281                  | 278     |

### Example 5

Heated at 1300-1325° C. for one minute—total heat cycle, four minutes—end quenched for five minutes with 750 cc./min. of water through  $\frac{1}{16}$ " outlet disposed  $\frac{1}{8}$ " below test specimen. A shield was used.

| Distance from end of rod | Diamond pyramid hardness |                      |         |
|--------------------------|--------------------------|----------------------|---------|
|                          | One side of rod          | Opposite side of rod | Average |
| $\frac{1}{16}$ "         | 437                      | 450                  | 443     |
| $\frac{3}{16}$ "         | 421                      | 433                  | 427     |
| $\frac{1}{4}$ "          | 401                      | 421                  | 411     |
| $\frac{3}{8}$ "          | 366                      | 394                  | 380     |
| $\frac{1}{2}$ "          | 360                      | 390                  | 375     |
| $\frac{5}{16}$ "         | 348                      | 383                  | 365     |
| $\frac{7}{16}$ "         | 348                      | 360                  | 354     |
| $\frac{9}{16}$ "         | 327                      | 360                  | 343     |
| 1"                       | 317                      | 342                  | 330     |
| $1\frac{1}{16}$ "        | 285                      | 314                  | 299     |
| $1\frac{3}{16}$ "        | 285                      | 294                  | 290     |
| $1\frac{7}{16}$ "        | 274                      | 294                  | 284     |
| 2"                       | 274                      | 274                  | 274     |

### Example 6

Heated at 1500° C. for one minute in a container having a pool of water in the bottom—total heat cycle, five minutes—quenched in the water at the bottom of the container.

| Distance from end of rod | Diamond pyramid hardness |                      |         |
|--------------------------|--------------------------|----------------------|---------|
|                          | One side of rod          | Opposite side of rod | Average |
| $\frac{1}{16}$ "         | 1,097                    | 1,081                | 1,089   |
| $\frac{3}{16}$ "         | 1,064                    | 870                  | 970     |
| $\frac{1}{4}$ "          | 960                      | 514                  | 734     |
| $\frac{3}{8}$ "          | 792                      | 514                  | 650     |
| $\frac{1}{2}$ "          | 627                      | 425                  | 525     |
| $\frac{5}{16}$ "         | 592                      | 425                  | 512     |
| $\frac{7}{16}$ "         | 548                      | 413                  | 478     |
| $\frac{9}{16}$ "         | 519                      | 413                  | 463     |
| 1"                       | 493                      | 413                  | 453     |
| $1\frac{1}{16}$ "        | 464                      | 413                  | 438     |
| $1\frac{3}{16}$ "        | 464                      | 383                  | 423     |
| $1\frac{7}{16}$ "        | 464                      | 366                  | 416     |
| $2\frac{1}{16}$ "        | 464                      | 366                  | 416     |
| $2\frac{3}{16}$ "        | 421                      | 366                  | 393     |
| $2\frac{5}{16}$ "        | 421                      | 366                  | 393     |
| $2\frac{7}{16}$ "        | 327                      | 322                  | 324     |
| 3"                       | 279                      | 274                  | 276     |

### Example 7

Heated at 1500° C. for one minute—total heat cycle, four minutes—cooled 12.5 minutes in argon with  $3\frac{1}{2}$ " of water in bottom of container.

| Distance from end of rod | Diamond pyramid hardness |                      |         |
|--------------------------|--------------------------|----------------------|---------|
|                          | One side of rod          | Opposite side of rod | Average |
| $\frac{1}{16}$ "         | 946                      | 1,033                | 991     |
| $\frac{3}{16}$ "         | 946                      | 1,132                | 1,039   |
| $\frac{1}{4}$ "          | 803                      | 960                  | 880     |
| $\frac{3}{8}$ "          | 613                      | 803                  | 713     |
| $\frac{1}{2}$ "          | 468                      | 548                  | 508     |
| $\frac{5}{16}$ "         | 421                      | 488                  | 451     |
| $\frac{7}{16}$ "         | 370                      | 488                  | 430     |
| $\frac{9}{16}$ "         | 366                      | 464                  | 416     |
| 1"                       | 345                      | 390                  | 367     |
| $1\frac{1}{16}$ "        | 342                      | 390                  | 367     |
| $1\frac{3}{16}$ "        | 309                      | 380                  | 345     |
| $1\frac{7}{16}$ "        | 309                      | 348                  | 325     |
| 2"                       | 274                      | 289                  | 281     |

### 4 Example 8

Heated at 1300° C. for one minute—total heat cycle, four minutes—cooled five minutes in argon that had been bubbled through water. The argon was introduced at the bottom of the test container so as to impinge on the end of the test rod.

| Distance from end of rod | Diamond pyramid hardness |                      |         |
|--------------------------|--------------------------|----------------------|---------|
|                          | One side of rod          | Opposite side of rod | Average |
| $\frac{1}{16}$ "         | 681                      | 734                  | 707     |
| $\frac{3}{16}$ "         | 734                      | 792                  | 763     |
| $\frac{1}{4}$ "          | 734                      | 792                  | 763     |
| $\frac{3}{8}$ "          | 734                      | 542                  | 642     |
| $\frac{1}{2}$ "          | 606                      | 483                  | 543     |
| $\frac{5}{16}$ "         | 572                      | 421                  | 495     |
| $\frac{7}{16}$ "         | 514                      | 366                  | 441     |
| $\frac{9}{16}$ "         | 483                      | 330                  | 405     |
| 1"                       | 437                      | 322                  | 377     |
| $1\frac{1}{16}$ "        | 409                      | 322                  | 367     |
| $1\frac{3}{16}$ "        | 366                      | 322                  | 343     |
| $1\frac{7}{16}$ "        | 336                      | 309                  | 322     |
| 2"                       | 322                      | 302                  | 312     |

The results of these tests are given graphically in the drawing. It is evident at a glance that the test samples heated in argon containing water vapor are much harder than those heated in argon which does not contain water vapor. Example 1 shows that heat treating a vanadium-20% titanium rod at 1525° C. for one minute does not greatly affect the hardness of the alloy. Similarly, end quenching samples which had been heated in an argon atmosphere which did not contain water vapor—see Examples 3, 4 and 5—increased the hardness only slightly. In Examples 2, 6, 7 and 8 the test samples were heated in an argon atmosphere containing water vapor and in every case the hardness of the alloy is greatly increased. It will be appreciated that the rapid decrease in hardness along the length of the test rods in some of the examples is due to the experimental approach. In Examples 2, 6 and 7 the rod was heated while disposed vertically in a container containing water. Thus there was a higher proportion of water vapor in the container at the lower end of the rod than at the top and, as expected, the lower end of the rod was harder than the upper end of the rod. In Example 8 argon saturated with water vapor was introduced into the bottom of the container so as to impinge on the bottom of the test rod. Examples 7 and 8 prove that the increased hardness is caused by the water vapor in the atmosphere, since increased hardness is obtained both by heating the test sample over water and by saturating the argon with water vapor before admitting it into the test container. Tests 2 and 6 prove that completely quenching the test sample in water does not adversely affect the hardness. It is noted that in both these examples the test samples were heated in argon while suspended over water and were then dropped into the water. It is believed that quenching the sample in water or some other inert liquid would be desirable, although this has not as yet been completely proved.

These tests taken together indicate that oxygen is added to the surface of the test sample when the test sample is heated in argon containing water vapor. Hardening then occurs upon cooling of the sample.

A maximum temperature of 1300° C. is specified because the grain size increases and plasticity and elongation suffer at higher temperatures. Temperatures lower than 1100° C. may be satisfactory; however, a longer time at temperature is needed.

It will be understood that the invention is not to be limited to the details given herein but that it may be modified within the scope of the appended claim.

The embodiments of the invention in which an exclusive property or privilege is claimed are defined as follows:

1. A method of casehardening a vanadium-20% titanium alloy comprising heating the alloy in argon saturated

in water at 1100-1300° C. for five minutes including four minutes to reach temperature.

## References Cited

## UNITED STATES PATENTS

2,217,802 10/1940 Koehring ----- 148—6.3X  
3,111,434 11/1963 Takao et al. ----- 148—13.1  
3,314,827 4/1967 Vries ----- 148—13.1

## OTHER REFERENCES

Z. Metallkde., vol. 57, 1966, pp. 66-69.  
Argonne National Laboratory—Report No. 6928, W. R. Burt et al., pp. 9-11, 68, 73-75.

5 CHARLES N. LOVELL, Primary Examiner

U.S. CL. X.R.

148—6.3, 31.5